

Charles Martin's Imp in reduction of Iron Ores

74397

PATENTED  
FEB 11 1868



# United States Patent Office.

CHARLES MARTIN, OF CHANCERY LANE, ENGLAND.

Letters Patent No. 74,897, dated February 11, 1868

## IMPROVEMENT IN THE REDUCTION OF REFRACTORY IRON ORES.

The Schedule referred to in these Letters Patent and making part of the same.

### TO ALL WHOM IT MAY CONCERN:

Be it known that I, CHARLES MARTIN, of Chancery Lane, in the county of Middlesex, England, have invented certain "Improvements in the Reduction of Refractory Iron Ores, and in the construction of furnaces to be employed for such purposes;" and I do hereby declare that the following is a full and exact description thereof, reference being had to the accompanying drawing, and to the letters of reference marked thereon.

The processes hitherto adopted for the treatment of what are known as "refractory" iron ores, in order to effect their reduction, have been slow and expensive, a large amount of fuel and a heavy pressure of blast having been always considered essential for such operations, whilst in the reduction of some ores, such as haematite or kidney ore, magnetic ore, and some others, it has been usual to facilitate the operation of smelting by the addition of ores of an inferior quality.

The present invention has for its object the reduction of such refractory ores in an unmixed state by means of a comparatively small amount of fuel and light pressure of blast.

It is not necessary that the ore should be calcined, and it should be reduced to fragments not exceeding a cubic inch in size, and it is also preferable to reduce the fuel to pieces of the size of an egg, or thereabouts. The fluxes employed are lime and clay, which latter substance has not hitherto been used in its simple state as a flux in iron-smelting. The lime should be free from sulphur and phosphorus, and should be reduced to fragments corresponding in size to those of the ore under treatment, and the clay should likewise be pure, dry, and in-particles.

Furnaces of the ordinary sizes are suited to the purposes of my said invention, but I prefer that they should be of a height equal to four times the diameter of the boshes; and in constructing a furnace expressly for these processes, the following proportions should be observed: The height should be four times the diameter of the boshes. The hearth should be one-third the diameter of the boshes, or rather less, in the proportion of three to ten, and one-fourth the diameter in depth; the boshes at an angle of seventy degrees from the boshes upwards, the inclination outwards being as one in fifty, but the upper part may be drawn in to two-thirds the diameter, for the convenience of the arrangement of the landing-stage, and of charging. The tuyeres should be six inches in diameter, and set about two and a half feet apart, a two-inch blast-pipe or tuyere being placed at the side of each of the ordinary tuyeres, and arranged diagonally to the bottom of the hearth. These I term the "diagonal" tuyeres, and are so placed that upon the blast being admitted through them to the molten metal, the latter is penetrated and moved in a continuous circular direction.

I prefer the use of cold blast, and especial care should be taken that no greater pressure is employed than is sufficient to penetrate the mass of fuel, ore, and fluxes. In small furnaces, a pressure of from one to two ounces per square inch is sufficient, an increased pressure to the amount, in some cases, of one pound per square inch, being used, according to the size of the furnace.

The furnace may be charged in the ordinary manner, and in the following order and proportions: Fuel, three parts; lime, three parts; clay, one part; and ore, nine parts. The proportions mentioned are necessarily approximative only, as variations therein may be desirable, according to the nature of the ore, as will be well understood by practical smelters.

The following precautions should be observed in the management of the furnace: When sufficient metal is in the hearth, the blast must be nearly turned off from the ordinary tuyeres, but the full working-pressure sufficient to penetrate the mass of fluid metal must be turned on to the "diagonal" tuyeres. The last-mentioned tuyeres should be so arranged as to be "bolted" in close to the hearth, and opened when the blast is applied, if necessary. Experience will determine the length of time the blast should be kept on, which will be usually from ten to twenty minutes, according to the mass of metal to be operated upon, the effect being the consumption of excess of carbon, thus refining and making it very limpid. The ingot-moulds should be loam-washed and heated to  $600^{\circ}$ , and, when filled, the metal therein should be worked up and down for a minute or two by a small rod, or pressure applied, to insure solidity; and the ingot so produced will be ready for the rolling-mill. If the blast is kept in longer than the time required, the metal will thicken, and subsequently "gob" up the furnace. Or it may be found preferable, after the blast has been on from the diagonal tuyeres a sufficient length of time, to clear the metal of slag, or rather to float it, to tap the metal into a ladle, and mix it there-

with a small portion of oxide of iron in a powdered state, the action of the oxygen contained therein being to combine with and remove the excess of carbon. The metal can then be poured into the ingot-moulds.

I will now proceed to refer to the annexed drawing, from which the mode of constructing blast-furnaces in accordance with my said invention will be clearly understood, such drawing being upon the scale of a quarter of an inch to a foot.

The brick-work of the furnace is surrounded with an iron casing, *m m*, shown at *A A*, the space between the casing and the brick-work being filled with sand. The iron casing is supported by columns, one of which is shown at *B*, thus allowing of the lower part of the furnace being removed and repaired without interfering with the upper portion. One of the ordinary tuyeres is shown at *a*, and one of the "diagonal" tuyeres at *b*. The other parts and form and proportions of the furnace are clearly shown by the drawing, and will be understood by persons acquainted with such structures, without special reference being made thereto.

Having thus described and ascertained the nature of my said invention, and the manner in which it is to be performed, I would observe, in conclusion, that what I consider novel and original, and therefore claim as constituting the invention hereinbefore described, are—

The methods of reducing refractory iron ores, and of constructing furnaces for such operations, as substantially hereinbefore described and set forth, or any mere modifications thereof.

CHARLES MARTIN.

Witnesses:

R. A. MORDAUNT VAUGHAN, 54 Chancery Lane,

M. WYNN, 24 Royal Exchange, London.